# EUROPEAN PATENT SPECIFICATION

(11) **EP 0 316 290 B1**
(45) Date of publication and mention of the grant of the patent: **15.07.1992**
(21) Application number: 88830478.9
(22) Date of filing: 08.11.1988
(51) Int. Cl.: H01T 13/41, H01C 7/00

(54) **A resistive mastic for sparking plugs with incorporated resistors**
Widerstandskitt für Zündkerzen mit eingebauten Widerständen
Mastic résistif pour bougies d'allumage à résistances incorporées

(30) Priority: 12.11.1987 IT 6796487
(43) Date of publication of application: 17.05.1989
(73) Proprietor: INDUSTRIE MAGNETI MARELLI S.p.A., 20128 Milano (IT)
(72) Inventor: Latte, Giovanni Michele, I-57100 Livorno (IT); Rossi, Roberto, I-20131 Milano (IT)
(74) Representative: Rambelli, Paolo

(56) References cited:
- DE-A- 3 226 340
- US-A- 4 006 106
- US-A- 4 112 330

## Description

The present invention relates to a resistive mastic for sparking plugs with incorporated resistors.

In order to screen sparking plugs to prevent the radiation of energy at a frequency which affects and prevents reception and transmission by radioelectrical equipment, it is known to use a mastic as a suppressor, the mastic being inserted in the insulating body between the central electrode and the current supply pin and sealing them as a result of its hot fusion.

The use of resistive mastics including components of glass, titanium dioxide and an organic binder is known from the literature. The resistance of such mastics varies greatly, however, when they are subjected to discharge at high tension and high temperature. It is possible to avoid these variations by means of stabilisation processes but these involve further operations, in addition to the normal production cycle, with a consequent increase in costs.

The particular object of the present invention is to produce a resistive mastic whose physical characteristics remain stable with time.

In view of this object, the subject of the invention is a resistive mastic characterised in that it comprises:
- a glass constituent based on boron and alkali metals silicate, constituted by:
a) a quantity of from 7 to 38% by weight of the total composition of the mastic of a low-melting glass having a dilatometric softening point between 500 and 600°C and a transformation temperature above 500°C,
b) a quantity of from 43 to 90% by weight of the composition of the mastic of a high-melting glass having a dilatometric softening point at least 100C degrees higher than that of the low-melting glass,
- a quantity of from 1 to 19% by weight of titanium dioxide and
- a first organic binder selected from the group consisting of dextrin, cellulose derivatives and vinyl alcohols in a quantity such as to give the mastic a resistivity value of no more than 20 Kohm and a second organic binder which has substantially no affect on the resistivity value.

In particular, a high-melting glass composition is selected which has a viscosity/temperature curve such that, during hot pressing, which is normally carried out at between 800 and 900°C, the glass remains substantially inert so as to create a structure which delimits the conductive mastic part which is normally interposed between the resistive mastic and the terminals of the central electrode and the core. The low-melting glass correspondingly has a viscosity/temperature curve such that it fuses completely at the hot pressing temperature, thus ensuring the compactness of the resistive mixture and good anchorage thereof to the ceramic body of the plug. Compositions which can be used for the two types of glass are shown in the table below by way of non-limiting example, expressed as percentages by weight.

It is preferable that the high-melting glass should have a lower total alkali metal oxide content than that of the low-melting glass.

The first organic binder is preferably constituted by dextrin, whose inclusion in the mastic composition causes an appreciable variation in its resistance, which is inversely proportional to the dextrin content. To give a stable resistance value, it is particularly preferred that the dextrin to titanium dioxide ratio should be within the range 0.06:1 to 0.23:1, and more preferably 0.09:1 to 0.15:1. The second binder, which does not affect the resistivity, is generally constituted by a wax emulsion.

According to another characterising aspect, the resistive mastic can be obtained by the mixing of:
i) a quantity of between 40 and 70% by weight of the total composition of the high-melting glass, with a particle size of between 0.2 and 0.4 mm,
ii) a quantity of between 20 and 55% by weight of the total composition of a mixture, previously ground to a particle size of less than 75 µm and including the low-melting glass, titanium dioxide and some of the high-melting glass,
iii) the quantities specified above of the first and second organic binders.

The mixture ii) preferably includes from 30 to 70% of low-melting glass; from 15 to 41% of high-melting glass and a quantity of from 5 to 35% by weight of titanium dioxide with a particle size of less than 10 µm, the percentages being percentages of the total quantity of the mixture ii).

The following example describes the preparation of a mastic composition according to the invention.

### Example

A glass B, having the composition given below, is milled to a particle size of between 5 and 15 µm

### Glass B

- SiO₂: 58.8% by weight
- B₂O₃: 22.5% by weight
- Al₂O₃: 8.5%
- CaO: 0.3%
- Na₂O: 5.6%
- K₂O: 2.8%

Transformation temperature 500°C.

Softening temperature 560°C.

The high-melting glass, having the composition given below, is then crushed and a fraction having a particle size of between 0.2 and 0.4 mm is selected.

### Glass A

- SiO₂: 64.0%
- B₂O₃: 25.0%
- Al₂O₃: 1.5%
- CaO: 6.0%
- MgO: 0.6%
- Li₂O: 2.6%
- Na₂O: 0.1%
- K₂O: 0.2%

Transformation temperature 545°C.

Softening temperature 700°C.

The following materials are then introduced into a vessel:
- glass B: 56%
- glass A less than 0.2 mm: 30%
- Titanium dioxide: 14%

The mixture thus obtained is then milled to a particle size of less than 75 µm.

45 parts by weight of high-melting glass and 5 parts by weight of wax emulsion are added to 49 parts by weight of the milled mixture. The mixture is pelletised by dampening with a solution of dextrin at a concentration such as to add 1% of dextrin, screened so as to obtain a fraction having a particle size of less than 0.75 mm, and dried in an oven at 120°C.

The mastic thus obtained is used as a resistive mass in sparking plugs with incorporated resistors, the mass being introduced into the insulator of the plug by conventional pressing techniques.

Tests carried out have shown, in particular, that the resistance is very stable when the plug is subjected to the following set of acceptance tests:
a) test discharging for 1 minute at 15 KV at ambient temperature, 3000 sparks/minute
b) heating at 350°C for 15 hours
c) test discharging at 15 KV, 300°C for 50,000,000 discharges at 50Hz.

In particular it was possible to confirm that the resistance and the stability thereof depend on the ratio of the dextrin to the titanium dioxide and on the quantities thereof relative to the total mass.

With reference to the resistive mastic-described in the example given above, the following variations in resistance, expressed as percentages of the initial value R_{O}, were found in the acceptance tests:
initial resistance R_{O} = 5.0 Kohm
- test a):: ΔR_{A}: ≦ 10% R_{O}
- test b):: ΔR_{B}: ≦ 10% R_{A}
- test c):: ΔR_{C}: ≦ 15% R_{A}

## Claims

1. A resistive mastic for sparking plugs with incorporated resistors, characterised in that it comprises:
- a glass constituent based on boron and alkali metals silicate, constituted by:
a) a quantity of from 7 to 38% by weight of the total composition of the mastic of a low-melting glass having a dilatometric softening point between 500 and 600°C and a transformation temperature above 500°C,
b) a quantity of from 43 to 90% by weight of the composition of the mastic of a high-melting glass having a dilatometric softening point at least 100C degrees higher than that of the low-melting glass,
- a quantity of from 1 to 19% by weight of titanium dioxide and
- a first organic binder selected from dextrin, cellulose derivatives and vinyl alcohols in a quantity such as to give the mastic a resistivity value of no more than 20 Kohm
and a second organic binder which has substantially no affect on the resistivity value.

2. A resistive mastic according to Claim 1, characterised in that the first organic binder is dextrin and in that the ratio by weight of the dextrin to the titanium dioxide is between 0.07:1 and 0.23:1.

3. A resistive mastic according to Claim 2, characterised in that the second organic binder is constituted by a wax emulsion.

4. A resistive mastic according to Claim 1 or Claim 2, characterised in that the high-melting glass has a lower alkali metal oxide content than that of the low-melting glass.

5. A resistive mastic according to any one of Claims 1 to 3, characterised in that it is obtainable by the mixing of:
i) a quantity of between 40 and 70% by weight of the total composition of the high-melting glass, with a particle size of between 0.2 and 0.4 mm,
ii) a quantity of between 20 and 55% by weight of the total composition of a mixture previously ground to a particle size of less than 75 µm and including the low-melting glass, titanium dioxide and some of the high-melting glass,
iii) the first and second organic binders.

6. A resistive mastic according to Claim 5, characterised in that the mixture ii) comprises from 30 to 70% of low-melting glass, from 15 to 40% by weight of high-melting glass and a quantity of from 5 to 35% by weight of titanium dioxide, the percentages being percentages of the total quantity of the mixture ii).

7. A resistive mastic according to any one of Claims 1 to 5, characterised in that the titanium dioxide has a particle size below 10 µm.

8. A sparking plug with an incorporated resistor, in which the resistor is constituted by a mastic according to any one of Claims 1 to 7.

## Patentansprüche

1. Widerstandskitt für Zündkerzen mit eingebauten Widerständen, dadurch gekennzeichnet, daß er folgendes umfaßt:
- einen Glasbestandteil auf der Grundlage von Bor und Alkalimetallsilikat, bestehend aus:
a) einer Menge von 7 bis 38 Gew.-%, bezogen auf die Gesamtzusammensetzung des Kitts, eines Glases mit niedrigem Schmelzpunkt, dessen dilatometrischer ErweichungSpunkt zwischen 500 und 600°C liegt und einer Transformationstemperatur oberhalb 500°C,
b) einer Menge von 43 bis 90 Gew.-%, bezogen auf die Zusammensetzung des Kitts, eines Glases mit hohem Schmelzpunkt, dessen dilatometrischer Erweichungspunkt mindestens 100°C höher ist als der des Glases mit niedrigem Schmelzpunkt,
- eine Menge von 1 bis 19 Gew.-% Titandioxid und
- ein erstes organisches Bindemittel, ausgewählt aus Dextrin, Zellulosederivaten und vinylalkoholen in einer Menge, die dem Kitt einen Widerstandswert von nicht mehr als 20 kohm verleiht, und
ein zweites organisches Bindemittel, welches im wesentlichen keine Auswirkung auf den Widerstandswert hat.

2. Widerstandskitt gemäß Anspruch 1, dadurch gekennzeichnet, daß das erste organische Bindemittel Dextrin ist und daß das Gewichtsverhältnis des Dextrins und des Titandioxids zwischen 0,07:1 und 0,23:1 liegt.

3. Widerstandskitt gemäß Anspruch 2, dadurch gekennzeichnet, daß das zweite organische Bindemittel aus einer Wachsemulsion besteht.

4. Widerstandskitt gemäß Anspruch 1 oder Anspruch 2, dadurch gekennzeichnet, daß das Glas mit hohem Schmelzpunkt einen geringeren Alkalimetalloxidgehalt hat als das Glas mit niedrigem Schmelzpunkt.

5. Widerstandskitt gemäß einem der Ansprüche 1 bis 3, dadurch gekennzeichnet, daß er durch das Mischen folgender Komponenten erhältlich ist:
i) einer Menge zwischen 40 und 70 Gew.-%, bezogen auf die Gesamtzusammensetzung, des Glases mit hohem Schmelzpunkt, mit einer Teilchengröße zwischen 0,2 und 0,4 mm,
ii) einer Menge zwischen 20 und 55 Gew.-%, bezogen auf die Gesamtzusammensetzung, einer Mischung, die vorher auf eine Teilchengröße von weniger als 75 µm gemahlen wurde und das Glas mit niedrigem Schmelzpunkt, Titandioxid und einen Anteil des Glases mit hohem Schmelzpunkt umfaßt,
iii) des ersten und des zweiten organischen Bindemittels.

6. Widerstandskitt gemäß Anspruch 5, dadurch gekennzeichnet, daß die Mischung ii) 30 bis 70 % des Glases mit niedrigem Schmelzpunkt, 15 bis 40 Gew.-% des Glases mit hohem Schmelzpunkt und eine Menge von 5 bis 35 Gew.-% Titan-dioxid umfaßt, wobei die prozentualen Anteile jeweils auf die Gesamtmenge der Mischung ii) bezogen sind.

7. Widerstandskitt gemäß einem der Ansprüche 1 bis 5, dadurch gekennzeichnet, daß das Titandioxid eine Teilchengröße von weniger als 10 µm hat.

8. Zündkerze mit eingebautem Widerstand, in der der Widerstand von einem Kitt gemäß einem der Ansprüche 1 bis 7 gebildet wird.

## Revendications

1. Un mastic résistif pour bougies d'allumage à résistances incorporées, caractérisé en ce qu'il comprend :
- un constituant de verre à base de bore et de silicate de métaux alcalins, constitvé de :
a) une quantité allant de 7 à 38 % en poids de la composition totale du mastic d'un verre à point de fusion bas ayant un point de ramollissement dilatométrique entre 500 et 600 °C et une température de transformation supérieure à 500 °C,
b) une quantité allant de 43 à 90 % en poids de la composition du mastic d'un verre à point de fusion élevé ayant un point de ramollissement dilatométrique supérieur d'au moins 100 degrés C à celui du verre à point de fusion bas,
- une quantité allant de 1 à 19 % en poids de dioxyde de titane et
- un premier liant organique choisi dans la dextrine, les dérivés de cellulose et les alcools vinyliques en une quantité permettant de conférer au mastic une valeur de résistivité non supérieure à 20 KOhm
et un second liant organique qui n'influe pratiquement pas sur la valeur de résistivité.

2. Un mastic résistif conforme à la revendication 1, caractérisé en ce que le premier liant organique est de la dextrine et en ce que le rapport pondéral entre la dextrine et le dioxyde de titane se situe entre 0,07:1 et 0,23:1.

3. Un mastic résistif conforme à la revendication 2, caractérisé en ce que le second liant organique est constitué d'une émulsion de cire.

4. Un mastic résistif conforme à la revendication 1 ou à la revendication 2, caractérisé en ce que le verre à point de fusion élevé présente une teneur en oxyde de métal alcalin inférieure à celle du verre à point de fusion bas.

5. Un mastic résistif conforme à l'une quelconque des revendications 1 à 3, caractérisé en ce qu'il est obtenu en mélangeant :
i) une quantité comprise entre 40 et 70 % en poids de la composition totale du verre à point de fusion élevé, avec une dimension de particules comprise entre 0,2 et 0,4 mm,
ii) une quantité comprise entre 20 et 55 % en poids de la composition totale d'un mélange broyé auparavant en une dimension de particules inférieure à 75 µm et comprenant le verre à point de fusion bas, du dioxyde de titane et une partie du verre à point de fusion élevé,
iii) les premier et second liants organiques.

6. Un mastic résistif conforme à la revendication 5, caractérisé en ce que le mélange ii) comprend de 30 à 70 % de verre à point de fusion bas, de 15 à 40 % en poids de verre à point de fusion élevé et une quantité allant de 5 à 35 % en poids de dioxyde de titane, les pourcentages étant des pourcentages de la quantité totale du mélange ii).

7. Un mastic résistif conforme à l'une quelconque des revendications 1 à 5, caractérisé en ce que le dioxyde de titane présente une dimension de particules inférieure à 10 µm.

8. Une bougie d'allumage à résistance incorporée, dans laquelle la résistance est constituée d'un mastic conforme à l'une quelconque des revendications 1 à 7.
